

## 1

2,980,517

## STABILIZATION OF FUEL OILS

Ira Kukin, Bronx, N.Y., and Kurt S. Spiegler, Pittsburgh, Pa., assignors to Gulf Research & Development Company, Pittsburgh, Pa., a corporation of Delaware

No Drawing. Filed May 31, 1957, Ser. No. 662,584

7 Claims. (Cl. 44—62)

This invention relates to stabilization of blended distillate fuel oils. More particularly, the invention relates to stabilization of mixtures of catalytically cracked and straight run fuel oil distillates during storage at ambient atmospheric temperatures.

Uncompounded distillate fuel oil compositions are often troublesome with regard to sludge deposition and color degradation during storage at normal atmospheric temperatures. Sludge deposits in distillate fuel oils are objectionable in that such deposits can cause clogging of burner filters, screens, nozzles, etc., and thereby lead to improper functioning of the combustion apparatus in which the fuel oil is consumed.

Although sludge deposition sometimes occurs in straight run distillate fuel oils and frequently occurs to a substantial degree in catalytically cracked fuel oil distillates, sludge deposition in blends of straight run and catalytically cracked fuel oil distillates presents an entirely distinct problem from that encountered with either component oil. While the sludge formed in such blended oils probably contains some sludge of the type formed by each component oil, the sludge formed in blended fuel oils is of different composition and is consistently greatly in excess of the amount that can be accounted for from the known sludging tendencies of the individual component oils.

It has heretofore been proposed to inhibit sludge deposition from mixed distillate fuel oils by incorporation therein of oil-soluble chemical inhibitors which are consumed during combustion of the oil.

It has now been found that sludge deposition in such mixed oils can be greatly alleviated by maintaining the oil in contact with an oil-insoluble inhibitor during storage, which inhibitor can be used repeatedly and which is not consumed during combustion. The present invention, based on this discovery, relates to a process for improving the stability of mixed, catalytically cracked and straight run distillate fuel oils, and particularly to improving the stability of the mixed oils with respect to sludge deposition in order to improve the appearance of such oils and to render them more effective for use in fuel oil furnaces and the like, even after being stored for extended periods. We have found that improved storage stability in the mixed distillate fuel oils can be obtained by maintaining the mixed oils during storage at ambient atmospheric temperatures in contact with a sludge-inhibiting proportion of an oil-insoluble, strongly basic, anion exchange resin. Strongly basic anion exchange resins comprise a polymeric matrix having a plurality of quaternary ammonium hydroxide groups associated therewith. Typical of the class are resins comprising the hydroxide form of a tertiary amine-quaternized, haloalkylated copolymer of about 80 to 99.9 percent of a monovinyl aromatic hydrocarbon and about 0.1 to 20 percent of a divinyl aromatic hydrocarbon. We have also found that the moisture content of the resin is important insofar as the stability of the fuel oil is concerned. For best results the resin should contain at least about 25 percent water, and preferably from about 35 percent water up to the point of saturation. Copolymers containing 0.5 to 6 percent divinyl aromatic hydrocarbons are particularly valuable because of their

## 2

reduced fouling tendencies and greater exchange capacities in fuel oils. By way of example, excellent results are obtainable with a strongly basic anion exchange resin that comprises the hydroxide form of a dimethyl ethanol amine-quaternized, chloromethylated copolymer of about 99 percent styrene and about 1 percent divinyl benzene, that contains about 55 percent moisture. Copolymers of other monovinyl and divinyl aromatic hydrocarbons can be used. For example, monovinyl aromatic hydrocarbons 10 capable of forming copolymers within the scope of the invention are typified by the following: styrene, ortho-, meta- and para-methyl styrenes, ortho-, meta- and para-ethyl styrenes, vinyl naphthalene, vinyl anthracene, and their homologues. Examples of divinyl aromatic hydrocarbons 15 that can form copolymers included within the scope of the invention include divinyl benzene, divinyl toluenes, divinyl naphthalene, divinyl ethyl benzenes, divinyl xylenes, and their homologues. An example of a preferred haloalkyl group is the chloromethyl group. Examples 20 of other haloalkyl groups include chlorobutyl, bromoethyl, and the like. Preferred tertiary amine quaternizing agents include dimethyl ethanol amine and trimethyl amine. Other suitable quaternizing agents include triethyl and tripropyl amines, dimethyl ethyl amine, diethyl cyclohexyl amine, tricyclohexyl amine, triphenyl amine, diphenyl ethyl amine, benzyl dimethyl amine, benzyl phenyl methyl amine, methyl diethanol amine, methyl ethyl propanol amine, etc. Additional examples 25 of resins included by the process of this invention include the hydroxide form of a diethyl cyclohexyl amine-quaternized chlorobutylated copolymer of 96 percent meta-methyl styrene and 4 percent divinyl benzene, and the hydroxide form of a benzyl phenyl methyl amine-quaternized bromoethylated copolymer of 94 percent 30 vinyl naphthalene and 6 percent divinyl xylene, each in a moisture saturated condition.

The predominant non-crosslinked portion of the chloride form of a tertiary amine-quaternized haloalkylated copolymer of vinyl and divinyl aromatic hydrocarbons, for example, a trimethyl amine-quaternized chloromethylated copolymer of styrene and divinyl benzene can be represented by the following structural formula:



50 whereas the crosslinked portion can be represented as follows:



In the hydroxide form, the chlorine atoms are substituted 60 with hydroxyl groups in the above structures.

It has not been determined exactly in what way the 65 strongly basic anion exchange resins function to improve the stability of the mixed fuel oils. Accordingly, the invention is not limited to any particular theory of operation. It might appear that the strongly basic anion exchange resins act to remove impurities of a non-hydrocarbon nature, such as mercaptans, naphthenic acids, phenols, etc., from the oil. However, this possibility is more or less negated by the fact that mere percolation 70 of the fuel oil through a bed of a strongly basic anion exchange resin fails to improve the stability of the oil. Also, it has been found that fuel oil samples treated ac-

cording to the method of this invention showed no significant changes, as compared with an untreated sample of the same oil, when tested for total sulfur, nitrogen, mercaptans, pyrroles, peroxides, and water content. A more plausible explanation for the effectiveness of the anion exchange resins in stabilizing the blended fuel oils may be that the anion exchange resins act to remove sludge and color precursors as they are formed. The sludge and color precursors may in and of themselves form sludge and color bodies, or they may merely catalyze formation of sludge and color bodies. The anion exchange resins definitely do not function as sludge dispersants, as they are entirely insoluble in fuel oil.

The resin:oil proportions that are effective for the purposes of this invention will vary primarily according to the degree of contact between the resin and the fuel oil. The commercial resins as purchased, before conversion to the hydroxide form, are normally in comminuted form, in the shape of small granules or beads of relatively large surface area. For this reason, the degree of interfacial contact between oil and resin is potentially large, particularly in the case of the porous resin particles. Under comparatively static storage conditions we have found that excellent results can be obtained by more or less centrally suspending as little as about 0.2 to 2 percent resin by weight of the oil in the stored oil. Inasmuch as resins have been found unexhausted when used in such proportions after extended contact with stored fuel oil, substantially smaller proportions can be used. For example, an improvement in stability can be obtained using as little as about 0.004 weight percent resin, particularly where the oil or the resin is circulated to improve the interfacial contact. Normally, about 0.05 to 5 weight percent resin will effect a substantial improvement in the stability of the oil. Since the anion exchange resins are oil-insoluble, there is no need, other than as may be imposed by practical considerations, to restrict the maximum proportion of the resin. However, from a practical standpoint, it will normally be undesirable to employ more than about 10 percent resin by weight of the oil.

The desired intercontact between oil and resin can be obtained in any convenient way in the storage containers. For example, one or a number of oil-permeable containers containing small portions of the resin can be suspended at suitably spaced locations in the oil. Alternatively, permeable containers containing the resin can be suspended from a plurality of radially disposed arms which can be rotated continuously or intermittently to obtain the desired intercontact. Suitable permeable containers have been prepared from muslin, linen and nylon fabric (woven and unwoven) and from stainless steel screen. Another way of obtaining the desired intercontact is to circulate the oil from the main storage vessel through a bypass containing the resin. Still another method is to provide a lining for the storage vessels having the anion exchange resin particles disposed thereon. Also, sheets or strips of oil-resistant material, e.g., plastic, having anion exchange resin particles adhering thereto can be suspended in the oil during storage. The resin in finely divided form, so as to minimize settling, can also be metered into the oil as it is pumped into the storage container and recovered from the oil by filtration as the oil is removed from storage.

While the invention can be used in large storage vessels of the type employed in petroleum refineries, it is well-adapted for use in the smaller tanks of jobbers or individual consumer installations, and especially for use in transport vessels, e.g., tank cars, etc., since the movement of such vessels provides efficient intercontact of the ion-exchange resin and the oil.

As the anion exchange resins continue to be maintained in contact with stored fuel oils, they tend to become exhausted, and therefore to become less effective stabilizers. When the resins are no longer capable of main-

taining the desired stability in the fuel oils, or at any time before this point has been reached, the resins can be regenerated by treatment with aqueous caustic, that is, sodium hydroxide. The method of regenerating spent anion exchange resins with aqueous caustic is conventional and need not be described in detail here.

The stability problem with which the present invention is concerned exists when a catalytically cracked and a straight-run oil are combined in such proportions as to cause a substantial, combined sludging effect of the type described above. The invention is important when the ratio of the volume of the catalytically cracked oil to the straight run oil is within the range of 9:1 to 1:9. The invention is especially advantageous when applied to mixed fuel oils containing these oils in a volume ratio within the range of 4:1 to 1:4.

In order to demonstrate the effectiveness in mixed distillate fuel oils of strongly basic anion exchange resins of the class disclosed above, various tests were carried out, including a light stability test and a long term storage test. The light stability test was carried out by exposing a 4 oz. sample of oil to be tested to a light source rich in ultraviolet rays, for periods of 4 hours alternated with periods of 7 hours, during which the oil was stored in the dark. The test was completed after 72 hours' exposure to the light. Visual estimates were made of the sludge and color after each complete, eleven-hour, "on-off" cycle. The exposure to light was accomplished by putting samples of fuel oil in 4 oz. flint glass bottles. These bottles were placed in an enclosure adjacent a light source which was a Hanovia, S2353 "L" type burner, Analytical Model quartz lamp. The light source was made intermittent by passing light from the above lamp through a rotating, slotted drum. A Corning polished glass filter No. 9863 (2400-4000 angstroms) was interposed between the light source and the oil sample bottles. The speed of the rotating drum was 1 revolution in 3 seconds. The evenly spaced, light-transmitting slits were 8 mm. wide and 110 mm. in height. The distance between slits was 37 mm. The sample holder was so arranged that each sample bottle was irradiated by light of 12 foot candles intensity. This arrangement permitted accelerated fuel oil aging at a temperature which never exceeded 80° F. The effect of the exposure to light was judged by swirling the bottle and estimating the quantity of precipitate which had settled. This was recorded as Trace, Light, Medium or Heavy. Seventy-two hours' exposure under the conditions of this test correspond approximately to 1½ to 2 years of normal storage in actual usage.

The long term storage stability test was carried out by pouring 1500 ml. of the fuel to be tested into a two-quart Mason jar and immersing an 8" x 1½" x 1/32" SAE 1020 cold rolled steel strip in the oil. The steel surface to oil ratio approximates that existing in a 55 gallon steel drum. The jar was then closed with a vented lid and was stored in total darkness at ambient atmospheric temperature. Periodic sampling and testing were carried out as rapidly as possible in subdued light. The extent of deterioration of the fuel was determined by the amount of precipitate observed and designated as Trace, Light, Medium or Heavy. Any staining or corrosion of the steel strip was noted.

In the following table there are given the results of light stability and storage tests made on mixed fuel oils of the character indicated, both in the absence of a resin, and in contact with a strongly basic anion exchange resin of the class disclosed above. The resin employed in these tests is adequately identified as the hydroxide form of a porous, quaternized chloromethylated copolymer of about 97 percent styrene and about 3 percent divinyl benzene, that has been quaternized with dimethyl ethanol amine. The chloride form of a resin essentially identical with the foregoing is marketed as "Amberlite IRA 411." The chloromethylated copolymer, as such, contained in

excess of 2 percent chlorine. The hydroxide form of the resin used in the tests was prepared by placing the corresponding chloride form of the resin in a chromatographic tube to a depth such that the height to diameter ratio of the resin column was approximately 10 to 1. The resin was then washed with 10 times its volume of a solution of 8 percent sodium hydroxide, which was followed with distilled water washing until the eluate was no longer basic. The resin was then dried under vacuum for 3 hours. The relatively dry resin then was suitably hydrated by stirring in a container with an excess of water for 15 minutes. After decanting the excess water the resin was filtered through a Büchner funnel (under suction) to remove surface water. The moist resin, prepared essentially as indicated, was then placed in a permeable, muslin container and the latter was substantially centrally suspended by a cord in the fuel oils. The hydroxide form of the resin as prepared above is referred to hereinafter as Resin A.

## Total exchange capacity:

|                    |      |
|--------------------|------|
| Meq./ml. wet resin | 0.7. |
| Meq./g. dry resin  | 3.0. |

Typical wet screen analysis  
(U.S. standard screens)

## Size of mesh:

|    |      |
|----|------|
| 20 | 19.1 |
| 30 | 44.2 |
| 40 | 29.3 |
| 50 | 6.9  |
| 70 | 0.5  |

Fines content: Less than 2%.

15 No. 2 fuel oil distillate is defined in the ASTM Standards on Petroleum Products and Lubricants for 1956 under the designation D396-48T.

The following Table I presents the data obtained in the light stability tests:

TABLE I

|                                                                                                                                                                            | Blend A | Example I | Blend B    | Example II | Example III               |
|----------------------------------------------------------------------------------------------------------------------------------------------------------------------------|---------|-----------|------------|------------|---------------------------|
| <b>Sample Make-up:</b>                                                                                                                                                     |         |           |            |            |                           |
| Fuel Oil Blend, Vol. Percent—                                                                                                                                              |         |           |            |            |                           |
| A. 31.3% West Texas, Doctor-Sweetened, Straight Run No. 2 Fuel Oil Distillate; 21.3% Virgin S. R. No. 2 Fuel Oil Distillate; 47.4% Cat. Cracked No. 2 Fuel Oil Distillate. | 100.    | 100.      |            |            |                           |
| B. 31.3% West Texas, Doctor-Sweetened, No. 2 Fuel Oil Distillate; 21.3% Virgin S. R. No. 2 Fuel Oil Distillate; 47.4% Cat. Cracked No. 2 Fuel Oil Distillate.              |         |           | 100.       | 100.       | 100.                      |
| Ion-Exchange Resin A in Contact with Fuel Oil—<br>G./100 Ml.                                                                                                               |         | 2.        |            | 2.         | 2.                        |
| Wt. Percent                                                                                                                                                                |         | 2.3.      |            | 2.3.       | 2.3.                      |
| Water Saturation of Resin A, Wt. Percent                                                                                                                                   |         | 65.       |            | 60.        | 35.                       |
| <b>Inspections:</b>                                                                                                                                                        |         |           |            |            |                           |
| Color, ASTM Union                                                                                                                                                          | 2—      | 2—        | 2—         | 2—         | 2—                        |
| Gravity, ° API                                                                                                                                                             | 33.2    |           | 33.7       |            |                           |
| Specific Gravity, 60°/60° F                                                                                                                                                | 0.8501  |           | 0.8565     |            |                           |
| Neutralization Value—                                                                                                                                                      |         |           |            |            |                           |
| Total Acid Number                                                                                                                                                          | 0.01    | 0.01      | 0.02       | 0.02       | 0.02                      |
| Total Base No.                                                                                                                                                             | 0.13    | 0.13      | 0.09       | 0.09       | 0.09                      |
| Stability Test, Intermittent Ultraviolet Light:<br>Glass Container, After Exposure to Light, Appearance                                                                    | Stained | Clear     | Stained    | Clear      | Trace of Stain on Bottom. |
| Qualitative Estimate of Sludge—                                                                                                                                            |         |           |            |            |                           |
| 36 Hours                                                                                                                                                                   | Medium+ | Trace+    | Medium+    | Trace+     | Trace+                    |
| 72 Hours                                                                                                                                                                   | Heavy   | Light     | Very Heavy | Light+     | Heavy.                    |
| Color, ASTM Union                                                                                                                                                          | 4       | 3         | 4          | 3.5        | 3.5                       |

The corresponding chloride form of the commercial resin has the following characteristics:

|                                                   |                                     |
|---------------------------------------------------|-------------------------------------|
| Physical form                                     | Uniform, bead-like porous particles |
| Density as supplied, lbs. per cu. ft.             | 41.                                 |
| Moisture content as supplied, percent             | 53-63.                              |
| Screen grading (wet) mesh (U.S. standard screens) | 20-50.                              |
| Effective size, mm.                               | 0.35-0.50.                          |

50

55 Resin A.

It will be seen from the foregoing table that a strongly basic anion exchange resin of the class disclosed will effect a substantial improvement in the stability of mixed catalytically cracked and straight run fuel oil distillates. It will also be seen that the stability imparted by contact with the resin is reduced when using a resin of relatively lower moisture content.

In the following Table II there are tabulated the results obtained in the long term storage tests carried out on a mixed distillate fuel oil alone and stored in contact with

TABLE II

|                                                                                                                                                                 | Blend C         | Example III   |
|-----------------------------------------------------------------------------------------------------------------------------------------------------------------|-----------------|---------------|
| <b>Sample Make-Up:</b>                                                                                                                                          |                 |               |
| Fuel Oil Blend, Vol. Percent—                                                                                                                                   |                 |               |
| C. 33.3% Doctor-Sweetened W.T.S.R. No. 2 Fuel Oil Distillate; 33.3% Coastal S.R. No. 2 Fuel Oil Distillate; 33.3% Fluid Cat. Cracked No. 2 Fuel Oil Distillate. | 100.            | 100.          |
| Resin A—                                                                                                                                                        |                 |               |
| Grams per 1500 Ml. Fuel Oil                                                                                                                                     |                 | 3.            |
| Weight Percent                                                                                                                                                  |                 | 0.2.          |
| Moisture Content of Resin, Wt. Percent (Approx.)                                                                                                                |                 | 50.           |
| Storage Stability Test:                                                                                                                                         |                 |               |
| After 6 months—                                                                                                                                                 |                 |               |
| Existen Insolubles (Visual)                                                                                                                                     | Heavy           | Light.        |
| Steel Strip, Appearance                                                                                                                                         | Stained         | Slight Stain. |
| Existen Insolubles, Mg./100 Ml.                                                                                                                                 | 8.4             | 3.8.          |
| Color, ASTM Union                                                                                                                                               | 3—              | 2.5—          |
| After 1 year—                                                                                                                                                   |                 |               |
| Existen Insolubles (Visual)                                                                                                                                     | Heavy           | Medium-+.     |
| Steel Strip, Appearance                                                                                                                                         | Heavily Stained | Slight Stain. |
| Existen Insolubles, Mg./100 Ml.                                                                                                                                 | 14.3            | 2.6.          |
| Color, ASTM Union                                                                                                                                               | 4.5             | 3—            |

From the data presented in the foregoing table it will be apparent that mixtures of catalytically cracked and straight run fuel oil distillates are stabilized by maintenance in contact during storage with a strongly basic anion exchange resin. It will be understood that the present invention is not limited to the specific embodiments given herein, and that other distillate fuel oil blends and other strongly basic anion exchange resins of the class disclosed herein can be substituted for the corresponding substances in the specific examples in the same or equivalent proportions. For example, for Resin A there can be substituted the water-saturated, hydroxide form of a porous, trimethyl amine-quaternized chloromethylated copolymer of about 97 percent styrene and about 3 percent divinyl benzene, or the saturated hydroxide form of a trimethyl amine-quaternized chloromethylated copolymer of 97.5 percent styrene, 1 percent divinyl benzene, and 1.5 percent ethyl styrene, and the like. Examples of commercial quaternary ammonium type resins that can be used include, in addition, to "Amberlite IRA 411," "Amberlite IRA 400," "Amberlite IRA 401," "Amberlite IRA 410," "Dowex 1" and "Dowex 2."

As another example of the practice of our invention, 3000 grams of a moisture saturated, trimethyl amine-quaternized chloromethylated copolymer of 96 percent styrene and 4 percent divinyl benzene, in the hydroxide form, prepared from the commercially obtained corresponding chloride form as described in connection with Resin A, is suspended in ten equal portions in muslin bags at about equally spaced locations near the bottom of a cylindrical, 500 gallon storage tank to which there is added 500 gallons of fresh, No. 2 fuel oil (50-50 by volume straight run and catalytically cracked distillate). After six months at ambient conditions, the tank is emptied. The resin is collected and after removal of adhering fuel oil, the resin is regenerated with ten times its volume of 8 percent aqueous sodium hydroxide, water washed, and returned while wet to the tank for further use.

All of the resins disclosed are regeneratable by treatment with dilute caustic, for example, by the same procedure described in connection with the generation of resin A from its corresponding chloride form.

The use of strongly basic, anion exchange resins is essential to the invention. Thus, for example, when a weakly basic, oil-insoluble, anion exchange material, calcium hydroxyapatite, in the proportion of about 2 grams per 1500 ml. of oil, was suspended in a run-of-the-refinery, mixed distillate fuel oil and subjected to the long term storage stability test, both the uninhibited and the inhibited oil showed heavy sludge deposits after four months. The explanation for this is believed to reside in the fact that weakly basic anion exchange materials are insufficiently basic to react completely with all of the weakly acidic sludge and color precursors present in mixed distillate fuel oil. The resins of the class disclosed herein possess a basicity comparable to that of sodium hydroxide.

It is to be emphasized that the resins disclosed herein should be maintained in contact with the fuel oil during storage for as long as it is desired to maintain the stability of the oil. Mere once-through contacting the oil with the resin, as by percolation through a bed of the latter, is not sufficient. As a matter of fact, when this procedure was followed with fuel oil blend C and resin A, the treated oil was found to deposit more sludge than the untreated oil.

Proportions mentioned herein are by weight where not specified otherwise.

Strongly basic anion exchange resins may be defined as those which on titration in a concentrated potassium chloride water solution, e.g., an 0.5 normal solution, with an equivalent amount of hydrochloric acid, will show a titration curve like that of a strong base, such as sodium hydroxide. A weakly basic anion exchange resin,

on the other hand, is one which on titration under the same conditions will show a titration curve like that of a weak base, such as ammonium hydroxide.

If desired, there may be added to fuel oils of the class disclosed herein, preferably, but not necessarily, after storage in contact with the anion exchange resin, sludge inhibitors, oxidation inhibitors, corrosion inhibitors, ignition quality improvers, combustion improvers and/or other additives adapted to improve the oils in one or more respects.

Many modifications and variations of the invention as described herein will suggest themselves to those skilled in the art. Obviously, these can be resorted to without departing from the spirit or scope of the invention. Therefore, only such limitations should be imposed in the present invention as are indicated in the appended claims.

We claim:

1. A process for stabilizing fuel oil comprising maintaining a mixture of catalytically cracked and straight run fuel oil distillates that normally tends to deposit sludge during storage in contact with a minor proportion, sufficient to stabilize the oils, of a strongly basic anion exchange resin that comprises a polymeric matrix having a plurality of quaternary ammonium hydroxide groups associated therewith substantially throughout the period of storage of said mixture of oils at ambient atmospheric temperature, where the moisture content of the resin is at least about 25 weight percent.
2. A process for stabilizing fuel oil comprising maintaining a mixture of catalytically cracked and straight run fuel oil distillates that normally tends to deposit sludge during storage in contact with a minor proportion, sufficient to stabilize the oils, of a strongly basic anion exchange resin substantially throughout the period of storage of said mixture of oils at ambient atmospheric temperature, said resin being the hydroxide form of a tertiary amine-quaternized haloalkylated copolymer of about 80 to 99.9 percent of a monovinyl aromatic hydrocarbon and about 0.1 to 20 percent divinyl aromatic hydrocarbon, where the moisture content of the resin is at least about 25 weight percent.
3. The process of claim 2 where the copolymer contains about 0.5 to 6 percent divinyl aromatic hydrocarbon.
4. The process of claim 2 where the resin is maintained in contact with the oil in a plurality of locations in the oil.
5. A process for stabilizing fuel oil comprising maintaining a mixture of catalytically cracked and straight run fuel oil distillates that normally tends to deposit sludge during storage in contact with a minor proportion of a strongly basic anion exchange resin substantially throughout the period of storage of said mixture of oils at ambient atmospheric temperature, said resin being the hydroxide form of a tertiary amine-quaternized haloalkylated copolymer of about 94 to 99.5 percent of a monovinyl aromatic hydrocarbon and about 0.5 to 6 percent of a divinyl aromatic hydrocarbon, where the moisture content of the resin is at least about 35 percent, where the tertiary amine substituents each contain 1 to 7 carbon atoms, and where the haloalkyl group contains 1 to 4 carbon atoms.
6. The process of claim 5 where the tertiary amine is dimethyl ethanol amine and the haloalkyl group is chloromethyl.
7. The process of claim 5 where the tertiary amine is trimethyl amine and the haloalkyl group is chloromethyl.

References Cited in the file of this patent

UNITED STATES PATENTS

|           |                 |                |
|-----------|-----------------|----------------|
| 2,367,803 | Schindler       | Jan. 23, 1945  |
| 2,713,077 | Rieve           | July 12, 1955  |
| 2,718,489 | Coonradt et al. | Sept. 20, 1955 |
| 2,730,486 | Coonradt et al. | Jan. 10, 1956  |
| 2,831,799 | Coonradt et al. | Apr. 22, 1958  |